

## UNITED STATES PATENT OFFICE.

ALEXANDER L. FEILD, OF JACKSON HEIGHTS, NEW YORK, ASSIGNOR TO ELECTRO-METALLURGICAL COMPANY, A CORPORATION OF WEST VIRGINIA.

## PROCESS OF PREPARING SILICON-ZIRCONIUM ALLOYS OF REDUCED SILICON CONTENT.

No Drawing.

Application filed April 21, 1924. Serial No. 708,030.

*To all whom it may concern:*

Be it known that I, ALEXANDER L. FEILD, a citizen of the United States, residing at Jackson Heights, in the county of Queens and State of New York, have invented certain new and useful Improvements in Processes of Preparing Silicon-Zirconium Alloys of Reduced Silicon Content, of which the following is a specification.

10 The invention is a process of preparing silicon-zirconium alloys of reduced silicon-content. Typical alloys of the class contemplated are those in which a low carbon content is obtained by incorporating into 15 the alloy a percentage of silicon which exceeds the zirconium percentage.

United States Patent 1,425,572, issued on Aug. 15, 1922 to Frederick M. Becket, describes a method whereby alloys of this

20 class may be produced, it being understood that a low carbon content is desirable when the alloy is to be used for certain purposes, for example for addition to molten steel.

When the Becket alloy is to be added to 25 steels the silicon content of which is already at or near the permissible limit, the high silicon content of the alloy is objectionable, since too much silicon accompanies the zirconium into the steel bath. It 30 is the object of the present invention to reduce the silicon content of such alloys as those described in the Becket patent, and preferably to reduce the silicon percentage until it falls below the zirconium percentage, without destroying any of the 35 advantageous characteristics of the alloy.

This object is accomplished by treating the alloy with an alkaline solvent for silicon, such as a solution of a hydroxid or carbonate of an alkali metal or a hydroxid of an alkaline-earth metal.

The process can be carried out under a wide range of conditions, including the nature of the alkali, the concentration of its 45 solution, the proportion of alkali to alloy treated, the fineness of division of the alloy, the temperature during treatment, the composition of the alloy treated, and so forth.

Sodium hydroxid is a cheap alkali, and 50 may be used with excellent results. Ten to thirty per cent solutions are convenient, but both higher and lower concentrations may be used. A fifty per cent excess of alkali over that theoretically necessary to react

with the silicon which it is found possible 55 to remove is mentioned by way of example. When the alloy is finely powdered, as to pass a 100-mesh screen, before the alkali treatment, the removal of the silicon is expedited, but such a fine subdivision of the 60 alloy is by no means indispensable. Indeed it has been found that under some conditions the process can be successfully applied to alloy which has only been crushed to lumps, since these disintegrate under the 65 action of the silicon-extracting reagent. The process may be carried out at any usual temperature. As in other chemical reactions of the same general class, it is found that stronger solutions of alkali, larger excesses 70 of alkali, finer division of the alloy treated, and higher temperatures, expedite the silicon removal.

The following examples will illustrate the 75 process:

I. An alloy containing 43.9% Si, 35.14% Zr, and about 16% Fe, was suitably treated with a 20% solution of NaOH. The resulting product contained only 37.9% Si and 44.17% Zr.

II. One hundred grams of an alloy containing Si 47.60%, Zr 43.52%, and Fe 5.99%, was ground to pass a 100 mesh screen and slowly added to a 30% solution of caustic soda containing about 45 g. NaOH. 80 The alloy was left in the caustic solution held at 90° C. for one-half hour after the final addition. Twenty-one and a half grams of the alloy dissolved, including 0.2 grams of zirconium. The undissolved alloy 85 contained 55.13% Zr, 34.60% Si, and 5.74% Fe. The ratio of silicon to zirconium was thus reduced from 1.09 to 0.63.

Alloys such as those described in the Becket patent usually contain considerable 95 quantities of iron, though the iron content can be reduced by appropriate measures. I have found that a low iron content facilitates the removal of silicon by the described method. It is my present belief that the optimum iron content for a maximum removal of silicon by the herein-described process may be determined by the following computation: If the weight of zirconium in a charge of the original alloy is multiplied 100 by 0.6 and the product subtracted from the weight of silicon in the charge, then the weight of iron present should not ma-

terially exceed one-third of the differences so obtained.

The iron remains with the insoluble material after the alkali treatment. Where the final product is to be added to a steel bath, a content of metallic iron is of course immaterial. If desired, the iron can be removed completely or in part, as by leaching with a reagent such as dilute sulphuric acid which attacks the iron preferentially.

Under favorable conditions it is possible to remove so much silicon from alloys of the kind referred to that the percentage of silicon in the product obtained does not materially exceed six-tenths of the zirconium percentage.

I claim:

1. Process which comprises reducing a zirconium compound with a carbonaceous reducing agent, simultaneously liberating in 20 the same charge such a quantity of silicon that a low-carbon alloy containing more silicon than zirconium is produced, and then removing silicon from the alloy with an alkaline solvent for silicon.

2. Process according to claim 1 wherein the iron content of the original alloy is kept low, substantially as described.

In testimony whereof, I affix my signature.

ALEXANDER L. FEILD.